

# United States Patent [19]

Dohnomoto et al.

[11] Patent Number: 4,595,638

[45] Date of Patent: Jun. 17, 1986

[54] COMPOSITE MATERIAL MADE FROM MATRIX METAL REINFORCED WITH MIXED ALUMINA FIBERS AND MINERAL FIBERS

[75] Inventors: Tadashi Dohnomoto; Masahiro Kubo, both of Toyota, Japan

[73] Assignee: Toyota Jidosha Kabushiki Kaisha, Toyota, Japan

[21] Appl. No.: 734,654

[22] Filed: May 16, 1985

[30] Foreign Application Priority Data

Mar. 1, 1985 [JP] Japan ..... 60-040908

[51] Int. Cl. 4 ..... B32B 5/02; B32B 7/00

[52] U.S. Cl. ..... 428/614; 428/608; 428/610; 420/411; 420/408

[58] Field of Search ..... 428/614, 610, 608

[56] References Cited

U.S. PATENT DOCUMENTS

4,157,409 6/1979 Levitt et al. ..... 428/608  
4,223,075 9/1980 Harrigan et al. ..... 428/614  
4,457,979 7/1984 Donomoto et al. ..... 428/614

FOREIGN PATENT DOCUMENTS

56-23242 3/1981 Japan ..... 428/614

Primary Examiner—Veronica O'Keefe  
Attorney, Agent, or Firm—Oblon, Fisher, Spivak,  
McClelland & Maier

[57] ABSTRACT

This composite material includes reinforcing hybrid fiber mixture material in a matrix of metal which is aluminum, magnesium, copper, zinc, lead, tin, or an alloy having these as principal components. The hybrid fiber mixture is a mixture of alumina fiber material and mineral fiber material. The alumina fiber material has principal components of at least about 80% by weight of  $\text{Al}_2\text{O}_3$  and remainder substantially  $\text{SiO}_2$ . And the mineral fiber material has as principal components  $\text{SiO}_2$ ,  $\text{CaO}$ , and  $\text{Al}_2\text{O}_3$ , the content of  $\text{MgO}$  being less than or equal to 10% by weight, the content of  $\text{Fe}_2\text{O}_3$  being less than or equal to 5% by weight, and the content of other inorganic substances being less than or equal to 10% by weight, with the percentage of non fibrous particles being less than or equal to 20% by weight, and with the percentage of non fibrous particles with diameters greater than 150 microns being less than or equal to 7% by weight. The volume proportion of the reinforcing hybrid fiber material is at least 1%. The qualities of this composite material with regard to wear, wear on a mating member, and bending strength are good.

16 Claims, 12 Drawing Figures



FIG. 1



FIG. 3



FIG. 2



FIG. 4



FIG. 5



FIG. 6



FIG. 7



FIG. 8



FIG. 9



FIG. 10



FIG. 11



FIG. 12



**COMPOSITE MATERIAL MADE FROM MATRIX METAL REINFORCED WITH MIXED ALUMINA FIBERS AND MINERAL FIBERS**

**BACKGROUND OF THE INVENTION**

The present invention relates to a type of composite material which includes fiber material as reinforcing material embedded in a mass of matrix metal, and more particularly relates to such a type of composite material in which the reinforcing material is a mixture of alumina fiber material and mineral fiber material and the matrix metal is aluminum, magnesium, copper, zinc, lead, tin, or an alloy having one or more of these as principal component or components.

In the prior art, relatively low melting point metals such as aluminum, magnesium, copper, zinc, lead, tin, or alloys having one or more of these as principal component or components have been very popular for use as materials for members which are in sliding contact with mating members, because of their affinity for such mating members and their good frictional characteristics. However nowadays, along with increasing demands for higher mechanical performance, the conditions in which such materials are required to operate are becoming more and more harsh, and tribological problems such as excessive frictional wear and adhesion burning occur more and more often; in the extreme case, these problems can lead to seizure of a moving member. For instance, if a diesel engine with aluminum alloy pistons is run under extreme conditions, there may arise problems with regard to abnormal wear to the piston ring grooves on the piston, or with regard to burning of the piston and of the piston rings.

One effective means that has been adopted for overcoming these tribological problems has been to reinforce such a relatively low melting point metal or alloy by an admixture of reinforcing fibers made of some extremely hard material. Thus, various composite materials including fibrous materials of various kinds as reinforcing material have been proposed. The advantages of such fiber reinforced materials include improved lightness, improved strength, enhanced wear characteristics, improved resistance to heat and burning, and so on. In particular, such concepts are disclosed in Japanese Patent Laying Open Publications Ser. Nos. Sho 58-93948 (1983), Sho 58-93837 (1983), Sho 58-93841 (1983), and Sho 59-70736(1984), of all of which Japanese patent applications the applicant was the same entity as the assignee of the present patent application, and none of which is it intended hereby to admit as prior art to the present application except insofar as otherwise obliged by law. Further, for the fiber reinforcing material, there have been proposed the following kinds of inorganic fiber materials: alumina fiber material, alumina-silica fiber material, silicon carbide fiber material, silicon nitride fiber material, carbon fiber material, potassium titanate fiber material, and mineral fiber material; and for the matrix metal, aluminum alloy and various other alloys have been suggested. Such prior art composite materials are disclosed, for example, in the above cited Japanese Patent Laying Open Publications Ser. Nos. Sho 58-93837 (1983) and Sho 58-93841 (1983). Of these abovementioned reinforcing fiber materials, for superior wear resistance properties and relatively low cost, the alumina-silica type, that is to say, either alumina fibers or alumina-silica fibers, are preferred—see Japanese Patent Laying Open Publication Ser. No. Sho

58-93837 (1983) and the abovementioned Japanese Patent Laying Open Publication Ser. No. Sho 58-93841 (1983)—and, for extremely low cost, mineral fibers (see Japanese Patent Application Ser. No. Sho 59-219091 5 (1984)) are preferred. Again, in the case of these various Japanese patent applications, the applicant was the same entity as the assignee of the present patent application, and it is not intended hereby to admit any of them as prior art to the present application except insofar as 10 otherwise obliged by law.

However, in the case of using alumina fibers as the reinforcing material for a composite material, the problem arises that these alumina fibers are very expensive, and hence high cost for the resulting composite material is inevitable. This cost problem, in fact is one of the biggest current obstacles to the practical application of certain composite materials for making many types of actual components. On the other hand, in contrast to the above mentioned alumina fibers, so called alumina-silica fibers whose principal components are alumina and silica are very inexpensive, and have conventionally for example been used in quantity as heat insulation fibers, in which case, particularly in view of their handling characteristics, they are normally used in the amorphous crystalline form; therefore, if such alumina-silica fibers could satisfactorily be used as reinforcing fiber material for a composite material, then the cost could be very much reduced. However, the hardness of such alumina-silica type fibers is substantially less than that of alumina fibers, so that it is easy for the wear resistance of such a composite material to fall short of the optimum. Further, in the case of using these types of fibers as reinforcing fiber material for a composite material, since alumina-silica fibers, and particularly alumina-silica fibers in the amorphous crystalline phase, are structurally unstable, the problem tends to arise, during manufacture of the composite material, either that the wettability of the reinforcing fibers with respect to the molten matrix metal is poor, or alternatively, when the reinforcing alumina-silica fibers are well wetted by the molten matrix metal, that a reaction between them tends to deteriorate said reinforcing fibers. This can in the worst case so deteriorate the strength of the resulting composite material, due to deterioration of the strength of the fibers themselves, that unacceptable weakness results. This problem particularly tends to occur when the metal used as the matrix metal is one which has a strong tendency to form oxides, such as for example magnesium alloy.

In this connection, hardness in a resulting composite material is also a very desirable characteristic, and in the case that the reinforcing fiber material is relatively expensive alumina fiber material the question arises as to what crystalline structure for the alumina fiber material is desirable. Alumina has various crystalline structure, and the hard crystalline structures include the delta phase, the gamma phase, and the alpha phase. Alumina fibers including these crystalline structures include "Saffil RF" (this is a trademark) alumina fibers made by ICI KK, "Sumitomo" alumina fibers made by Sumitomo Kagaku KK, and "Fiber FP" (this is another trademark) alumina fibers made by the Dupont company, which are 100% alpha alumina. With the use of these types of reinforcing alumina fibers the strength of the composite material becomes very good, but, since these fibers are very hard, if a member made out of composite material including them as reinforcing mate-

rial is in frictional rubbing contact with a mating member, then the wear amount on the mating member will be increased. On the other hand, a composite material in which the reinforcing fiber material is alumina fibers with a content of from 5% to 60% by weight of alpha alumina fibers, such as are discussed in the above cited Japanese Patent Laying Open Publication Ser. No. Sho 58-93841 (1983), has in itself superior wear resistance, and also has superior frictional characteristics with regard to wear on a mating member, but in the same way as in the cases of composite materials with alumina fibers of the above crystalline structures as reinforcing fibers is expensive as compared to a composite material with alumina-silica fibers as the reinforcing fiber material. It is therefore very difficult to select a crystalline structure of alumina which allows a composite material made from alumina fibers with that structure to be superior in strength and also to be superior in wear resistance, while maintaining a reasonable cost level.

In contrast to the above, so called mineral fibers, of which the principal components are  $\text{SiO}_2$ ,  $\text{CaO}$ , and  $\text{Al}_2\text{O}_3$ , are very much less costly than the above mentioned other types of inorganic fibers, and therefore if such mineral fibers are used as reinforcing fibers the cost of the resulting composite material can be very much reduced. Moreover, since such mineral fibers have good wettability with respect to molten matrix metals of the types detailed above, and deleterious reactions with such molten matrix metals are generally slight, therefore, as contrasted with the case in which the reinforcing fibers are fibers which have poor wettability with respect to the molten matrix metal and undergo a deleterious reaction therewith, it is possible to obtain a composite material with excellent mechanical characteristics such as strength. On the other hand, such mineral fibers are inferior to the above mentioned other types of inorganic fiber with regard to strength and hardness, and therefore, as contrasted to the cases where the other types of inorganic fibers mentioned above are utilized, it is difficult to manufacture a composite material using mineral fibers as reinforcing fibers which has excellent strength and wear resistance properties.

#### SUMMARY OF THE INVENTION

The inventors of the present invention have considered in depth the above detailed problems with regard to the manufacture of composite materials, and particularly with regard to the use of alumina-silica fiber material or mineral fiber material as reinforcing material for a composite material, and as a result of various experimental researches (the results of some of which will be given later) have discovered that it is effective to use as reinforcing fiber material for the composite material a mixture of alumina fiber material and mineral fiber material. And, further, the present inventors have discovered that such a composite material utilizing a mixture of reinforcing fibers has vastly superior wear resistance to that which is expected from a composite material having only alumina fibers as reinforcing material, or from a composite material having only mineral fibers as reinforcing material. In other words, the present inventors have discovered that the properties of a such a composite material utilizing such a mixture of reinforcing fibers are not merely the linear combination of the properties of composite materials utilizing each of the components of said mixture on its own, but exhibit some non additive non linear synergistic effect by the combi-

nation of the reinforcing alumina fibers and the reinforcing mineral fibers.

Accordingly, the present invention is based upon knowledge gained as a result of these experimental researches by the present inventors, and its primary object is to provide a composite material including reinforcing fibers embedded in matrix metal, which has the advantages detailed above including good mechanical characteristics, while overcoming the above explained disadvantages.

It is a further object of the present invention to provide such a composite material, which utilizes an inexpensive combination of materials.

It is a further object of the present invention to provide such a composite material, which is cheap with regard to manufacturing cost.

It is a further object of the present invention to provide such a composite material, which is light.

It is a further object of the present invention to provide such a composite material, which has good mechanical strength.

It is yet a further object of the present invention to provide such a composite material, which has high bending strength.

It is yet a further object of the present invention to provide such a composite material, which has good machinability.

It is a yet further object of the present invention to provide such a composite material, which has good resistance against heat and burning.

It is a further object of the present invention to provide such a composite material, which has good wear characteristics with regard to wear on a member made of the composite material itself during use.

It is a yet further object of the present invention to provide such a composite material, which does not cause undue wear on a mating member against which a member made of said composite material is frictionally rubbed during use.

It is a yet further object of the present invention to provide such a composite material, which is not liable to cause scratching on such a mating member against which a member made of said composite material is frictionally rubbed during use.

It is a yet further object of the present invention to provide such a composite material, in the manufacture of which the fiber reinforcing material has good wettability with respect to the molten matrix metal.

It is a yet further object of the present invention to provide such a composite material, in the manufacture of which, although as mentioned above the fiber reinforcing material has good wettability with respect to the molten matrix metal, no deleterious reaction therebetween substantially occurs.

According to the present invention, these and other objects are accomplished by a composite material, comprising: (a) reinforcing material which is a hybrid fiber mixture material comprising: (a1) a substantial amount of alumina fiber material with principal components at least about 80% by weight of  $\text{Al}_2\text{O}_3$  and remainder substantially  $\text{SiO}_2$ ; and (a2) a substantial amount of mineral fiber material having as principal components  $\text{SiO}_2$ ,  $\text{CaO}$ , and  $\text{Al}_2\text{O}_3$ , the content of included  $\text{MgO}$  therein being less than or equal to about 10% by weight, the content of included  $\text{Fe}_2\text{O}_3$  therein being less than or equal to about 5% by weight, and the content of other inorganic substances included therein being less than or equal to about 10% by weight, with the percentage of

non fibrous particles included therein being less than or equal to about 20% by weight, and with the percentage of non fibrous particles with diameters greater than about 150 microns included therein being less than or equal to about 7% by weight; and (b) a matrix metal selected from the group consisting of aluminum, magnesium, copper, zinc, lead, tin, and alloys having these as principal components; wherein (c) the volume proportion of said hybrid fiber mixture material in said composite material is at least 1%.

According to such a composition according to the present invention, the matrix metal is reinforced with a volume proportion of at least 1% of this hybrid fiber mixture material, which consists of alumina fibers which are hard and stable and are cheaper for example than silicon carbide fibers, mixed with mineral fibers, which are even more cheap than alumina fibers, and which have good wettability with respect to these kinds of matrix metal and have little deteriorability with respect to molten such matrix metals. Since, as will be described later with regard to experimental researches carried out by the present inventors, the wear resistance characteristics of the composite material are remarkably improved by the use of such hybrid reinforcing fiber material, a composite material which has excellent mechanical characteristics such as wear resistance and strength, and of exceptionally low cost, is obtained. Also, since the percentage of non fibrous particles included in the mineral fiber material is less than or equal to about 20% by weight and also the percentage of non fibrous particles with diameters greater than about 150 microns included in said mineral fiber material is less than or equal to about 7% by weight, a composite material with superior strength and machinability properties is obtained, and further there is no substantial danger of abnormal wear such as scratching being caused to a mating member which is in frictional contact with a member made of this composite material during use, due to such non fibrous particulate matter becoming detached from said member made of this composite material.

Generally, alumina-silica type fibers may be categorized into alumina fibers or alumina-silica fibers on the basis of their composition and their method of manufacture. So called alumina fibers, including at least 70% by weight of  $\text{Al}_2\text{O}_3$  and not more than 30% by weight of  $\text{SiO}_2$ , are formed into fibers from a mixture of a viscous organic solution with an aluminum inorganic salt; they are formed by oxidizing firing at high temperature. Particularly when the included weight proportion of  $\text{Al}_2\text{O}_3$  is 80% or more, such alumina fibers are stable with regard to reaction with such molten matrix metals as detailed above, and are not subject to deterioration by chemical combination with said molten matrix metal. Therefore it is specified, according to the present invention, that the  $\text{Al}_2\text{O}_3$  content of the alumina fiber material included in the hybrid reinforcing fiber material for the composite material of the present invention should be greater than or equal to about 80% by weight, and that the remainder of said alumina fiber material should be substantially  $\text{SiO}_2$ .

Now, as mentioned above, there are various crystalline structures for alumina, and of these alpha alumina is the most stable form and is known for its hardness and high coefficient of elasticity. For example, alumina fibers sold as heat resistant material usually have an alpha alumina content (i.e., a weight proportion of alpha alumina as compared to the total weight content of

alumina in said alumina fibers) of at least 60%, for reasons of heat resistance and dimensional stability. From a consideration of the characteristics of alpha alumina and of alumina fibers including a high proportion of alpha alumina, with a composite material utilizing alumina fibers including alpha alumina as the reinforcing material and for example aluminum alloy as matrix material, it would be considered that, the higher was the content of alpha alumina in the reinforcing fiber material, the better would be the mechanical strength of the composite material, and the better would be the rigidity and the wear resistance thereof, but also the greater would be the wear on a mating element cooperating therewith and the worse the machinability would be expected to be. However, according to the results of the experimental research carried out by the present inventors, these expectations are not correct. In fact, it was found that, in the case that the alpha alumina content of the reinforcing fibers was in the range of from 5 to 60% by weight, and particularly in the case that the alpha alumina content of said reinforcing fibers was in the range of from 10 to 50% by weight, the wear resistance and the machinability of the composite material could be improved, and moreover the wear amount of a mating element could be reduced. Additionally, the above ranges were confirmed to give particularly desirable mechanical characteristics such as fatigue strength. Accordingly, according to a specialized characteristic of the present invention, it is considered to be preferable, in the composite material of the present invention, that said alpha alumina content of said alumina fiber material should be between about 5% and about 60%, and it is considered to be even more preferable that said alpha alumina content should be between about 10% and about 50%.

Mineral fiber is a generic name for artificial fiber material including rock wool (or rock fiber) made by forming molten rock into fibers, slag wool (or slag fiber) made by forming iron slag into fibers, and mineral wool (or mineral fiber) made by forming a molten mixture of rock and slag into fibers. Such mineral fiber generally has a composition of about 35% to about 50% by weight of  $\text{SiO}_2$ , about 20% to about 40% by weight of  $\text{CaO}$ , about 10% to about 20% by weight of  $\text{Al}_2\text{O}_3$ , about 3% to about 7% by weight of  $\text{MgO}$ , about 1% to about 5% by weight of  $\text{Fe}_2\text{O}_3$ , and up to about 10% by weight of other inorganic substances. These mineral fibers are generally produced by a method such as the spinning method, and therefore in the manufacture of such mineral fibers inevitably a quantity of non fibrous particles are also produced together with the fibers. These non fibrous particles are extremely hard, and tend to be large compared to the average diameter of the fibers. According to the results of experimental research carried out by the inventors of the present invention, particularly the very large non fibrous particles having a particle diameter greater than or equal to 150 microns, if left in the composite material produced, impair the mechanical properties of said composite material, and are a source of lowered strength for the composite material, and moreover tend to produce problems such as abnormal wear in and scratching on a mating element which is frictionally cooperating with a member made of said composite material, due to these large and hard particles becoming detached from the composite material. Also, such large and hard non fibrous particles tend to deteriorate the machinability of the composite material. Therefore, in the composite

material of the present invention, the total amount of non fibrous particles included in the mineral fiber material incorporated in the hybrid fiber material used as reinforcing material is required to be limited to a maximum of 20% by weight, and preferably further is desired to be limited to not more than 10% by weight; and the amount of such non fibrous particles of particle diameter greater than or equal to 150 microns included in said mineral fiber material incorporated in the hybrid fiber material used as reinforcing material is required to be limited to a maximum of 7% by weight, and preferably further is desired to be limited to not more than 2% by weight.

According to the results of further experimental researches carried out by the inventors of the present invention, a composite material in which reinforcing fibers are a mixture of alumina fibers and mineral fibers has the above described superior characteristics, and, when the matrix metal is aluminum, magnesium, copper, zinc, lead, tin, or an alloy having these as principal components, even if the volume proportion of the reinforcing hybrid fiber mixture material is around 1%, there is a remarkable increase in the wear resistance of the composite material, and, even if the volume proportion of said hybrid fiber mixture material is increased, there is not an enormous increase in the wear on a mating element which is frictionally cooperating with a member made of said composite material. Therefore, in the composite material of the present invention, the total volume proportion of the reinforcing hybrid fiber mixture material is required to be at least 1%, and preferably is desired to be not less than 2%, and even more preferably is desired to be not less than 4%.

According to the results of experimental research carried out by the inventors of the present invention, the effect of improvement of wear resistance of a composite material by using as reinforcing material a hybrid combination of alumina fibers and mineral fibers is, as will be described below in detail, most noticeable when the ratio of the volume proportion of said alumina fiber material to the total volume proportion of said hybrid fiber mixture material is between about 5% and about 80%, and particularly when said ratio is between about 10% and about 65%. Accordingly, according to another specialized characteristic of the present invention, it is considered to be preferable, in the composite material of the present invention, that said ratio of the volume proportion of said alumina fiber material to the total volume proportion of said hybrid fiber mixture material should be between about 5% and about 80%, and it is considered to be even more preferable that said ratio should be between about 10% and about 65%.

And, further according to the results of experimental research carried out by the inventors of the present invention, when the ratio of the volume proportion of said alumina fiber material to the total volume proportion of said hybrid fiber mixture material is relatively low, and the corresponding volume proportion of the mineral fibers is relatively high—for example, if the ratio of the volume proportion of said alumina fiber material to the total volume proportion of said hybrid fiber mixture material is from about 5% to about 40%—then, unless the total volume proportion of said hybrid fiber mixture material in the composite material is at least 2% and even more preferably is at least 4%, it is difficult to maintain an adequate wear resistance in the composite material. And further it is found that, if the total volume proportion of said hybrid fiber mixture

5  
10  
15  
20  
25  
30  
35

material becomes greater than about 35% and particularly if said total volume proportion becomes greater than about 40%, then the strength and the wear resistance of the composite material actually start to decrease. Therefore, according to another specialized characteristic of the present invention, it is considered to be preferable, in the composite material of the present invention, that the ratio of the volume proportion of said alumina fiber material to the total volume proportion of said hybrid fiber mixture material should be between about 5% and about 40%, and even more preferably should be between about 10% and about 40%; and that the total volume proportion of said hybrid fiber mixture material should be in the range from about 2% to about 40%, and even more preferably should be in the range from about 4% to about 35%.

Yet further, according to the results of experimental research carried out by the inventors of the present invention, whatever be the ratio of the volume proportion of said alumina fiber material to the total volume proportion of said hybrid fiber mixture material, if the total volume proportion of said mineral fiber material in the composite material exceeds about 20%, and particularly if it exceeds about 25%, then the strength and the wear resistance of the composite material are deteriorated. Accordingly, according to another specialized characteristic of the present invention, it is considered to be preferable, in the composite material of the present invention, regardless of the value of the ratio of the volume proportion of said alumina fiber material to the total volume proportion of said hybrid fiber mixture material, that the total volume proportion of said mineral fiber material in the composite material should be less than about 25%, and even more preferably that said total volume proportion should be less than about 20%.

With regard to the state of mutual mixing of the alumina fibers and the mineral fibers in the composite material of the present invention, if this mutual mixing is not even and thorough, then the strength and the wear resistance of the composite material will be caused to be uneven. Therefore, according to another specialized characteristic of the present invention, it is considered to be preferable, in the composite material of the present invention, that the alumina fibers and the mineral fibers which make up the hybrid reinforcing fiber material should be well and evenly mixed together.

With regard to the proper fiber dimensions, in order to obtain a composite material with superior mechanical characteristics such as strength and wear resistance, and moreover with superior friction wear characteristics with respect to wear on a mating element, the alumina fibers included as reinforcing material in said composite material should, according to the results of the experimental researches carried out by the inventors of the present invention, preferably have in the case of short fibers an average fiber diameter of approximately 1.5 to 5.0 microns and a fiber length of 20 microns to 3 millimeters, and in the case of long fibers an average fiber diameter of approximately 3 to 30 microns. On the other hand, since the mineral which is the material forming the mineral fibers also included as reinforcing material in said composite material has a relatively low viscosity in the molten state, and, since the mineral fibers are relatively fragile when compared with the alumina fibers, these mineral fibers are typically made in the form of short fibers (non continuous fibers) with a fiber diameter of about 1 to 10 microns and with a fiber length of about 10 microns to about 10 cm. Therefore, when the

55  
60  
65

availability of low cost mineral fibers is considered, it is desirable that the mineral fibers used in the composite material of the present invention should have an average fiber diameter of about 2 to 8 microns and an average fiber length of about 20 microns to about 5 cm. Moreover, when the method of manufacture of the composite material is considered, it is desirable that the average fiber length of the mineral fibers used in the composite material of the present invention should be about 100 microns to about 5 cm, and, in the case of the powder metallurgy method, should be preferably about 20 microns to about 2 mm.

#### BRIEF DESCRIPTION OF THE DRAWINGS

The present invention will now be described in terms of several preferred embodiments thereof, and with reference to the appended drawings. However, it should be understood that the description of the embodiments, and the drawings, are not any of them intended to be limitative of the scope of the present invention, since this scope is intended to be understood as to be defined by the appended claims, in their legitimate and proper interpretation. In the drawings, like reference symbols denote like parts and dimensions and so on in the separate figures thereof; spatial terms are to be understood as referring only to the orientation on the drawing paper of the relevant figure and not to any actual orientation of an embodiment, unless otherwise qualified; in the description, all percentages are to be understood as being by weight unless otherwise indicated; and:

FIG. 1 is a perspective view showing a preform made of alumina fibers and mineral fibers stuck together with a binder, said preform being generally cuboidal, and particularly indicating the non isotropic orientation of said fibers;

FIG. 2 is a schematic sectional diagram showing a mold with a mold cavity, and a pressure piston which is being forced into said mold cavity in order to pressurize molten matrix metal around the preform of FIG. 1 which is being received in said mold cavity, during a casting stage of a process of manufacture of the composite material of the present invention;

FIG. 3 is a perspective view of a solidified cast lump of matrix metal with said preform of FIG. 1 shown by phantom lines in its interior, as removed from the FIG. 2 apparatus after having been cast therein;

FIG. 4 is a graph in which, for each of eight test sample pieces A0 through A100 thus made from eight various preforms like the FIG. 1 preform, during a wear test in which the mating member was a bearing steel cylinder, the upper half shows along the vertical axis the amount of wear on the actual test sample of composite material in microns, and the lower half shows along the vertical axis the amount of wear on said bearing steel mating member in milligrams, while the volume proportion in percent of the total reinforcing fiber volume incorporated in said sample pieces which consists of alumina fibers is shown along the horizontal axis; and this figure also shows by a double dotted line a theoretical wear amount characteristic based upon the so called compounding rule;

FIG. 5 is a graph in which, for each of said eight test sample pieces A0 through A100, the deviation dY between the thus theoretically calculated wear amount and the actual wear amount is shown along the vertical axis in microns, and the volume proportion X in percent of the total reinforcing fiber volume incorporated in

said sample pieces which consists of alumina fibers is shown along the horizontal axis;

FIG. 6 is similar to FIG. 4, and is a graph in which, for each of six other test sample pieces B0 through B100 during another wear test, the upper half shows along the vertical axis the amount of wear on the actual test sample of composite material in microns, and the lower half shows along the vertical axis the amount of wear on the bearing steel mating member in milligrams, while the volume proportion in percent of the total reinforcing fiber volume incorporated in said sample pieces which consists of alumina fibers is shown along the horizontal axis; and also this figure again also shows by a double dotted line a theoretical wear amount characteristic;

FIG. 7 is similar to FIG. 5, and is a graph in which, for each of said six test sample pieces B0 through B100, the deviation dY between the thus theoretically calculated wear amount and the actual wear amount is shown along the vertical axis in microns, and the volume proportion X in percent of the total reinforcing fiber volume incorporated in said sample pieces which consists of alumina fibers is shown along the horizontal axis;

FIG. 8 is similar to the graphs of FIGS. 4 and 6, and is a graph in which, for each of seven other test sample pieces C0 through C100 during another wear test, the upper half shows along the vertical axis the amount of wear on the actual test sample of composite material in microns, and the lower half shows along the vertical axis the amount of wear on the bearing steel mating member in milligrams, while the volume proportion in percent of the total reinforcing fiber volume incorporated in said sample pieces which consists of alumina fibers is shown along the horizontal axis; and also this figure again shows by a double dotted line a theoretical wear amount characteristic;

FIG. 9 is similar to the graphs of FIGS. 5 and 7, and is a graph in which, for each of said seven test sample pieces C0 through C100, the deviation dY between the thus theoretically calculated wear amount and the actual wear amount is shown along the vertical axis in microns, and the volume proportion X in percent of the total reinforcing fiber volume incorporated in said sample pieces which consists of alumina fibers is shown along the horizontal axis;

FIG. 10 is similar to the graphs of FIGS. 4, 6, and 8, and is a graph in which, for each of seven other test sample pieces D0 through D100 during another wear test, the upper half shows along the vertical axis the amount of wear on the actual test sample of composite material in microns, and the lower half shows along the vertical axis the amount of wear on the bearing steel mating member in milligrams, while the volume proportion in percent of the total reinforcing fiber volume incorporated in said sample pieces which consists of alumina fibers is shown along the horizontal axis; and also this figure again also shows by a double dotted line a theoretical wear amount characteristic;

FIG. 11 is similar to the graphs of FIGS. 5, 7, and 9, and is a graph in which, for each of said seven test sample pieces D0 through D100, the deviation dY between the thus theoretically calculated wear amount and the actual wear amount is shown along the vertical axis in microns, and the volume proportion X in percent of the total reinforcing fiber volume incorporated in said sample pieces which consists of alumina fibers is shown along the horizontal axis; and

FIG. 12 is a graph relating to bending strength tests of seven other test samples E0 through E100, showing bending strength in kg/mm<sup>2</sup> along the vertical axis, and showing the volume proportion in percent of the total reinforcing fiber volume incorporated in said sample pieces which consists of alumina fibers along the horizontal axis, and also showing for comparison the bending strength of a comparison sample piece which is composed only of pure matrix metal without any reinforcing fibers.

mixture, said preform having dimensions of 80 by 80 by 20 millimeters, as shown in perspective view in FIG. 1, wherein it is designated by the reference numeral 1. As suggested in FIG. 1, the orientation of the alumina fibers 2 and of the mineral fibers 2a in these preforms 1 was not isotropic in three dimensions; in fact, the alumina fibers 2 and the mineral fibers 2a were largely oriented parallel to the longer sides of the cuboidal preforms 1, i.e. in the x-y plane as shown in FIG. 1, and were substantially randomly oriented in this plane; but the fibers 2 and 2a did not extend very substantially in the z direction as seen in FIG. 1, and were, so to speak, somewhat stacked on one another with regard to this direction. Finally, each preform was fired in a furnace at about 600° C., so that the silica bonded together the individual alumina fibers 2 and mineral fibers 2a, acting as a binder.

### DESCRIPTION OF THE PREFERRED EMBODIMENTS

The present invention will now be described with reference to the preferred embodiments thereof, and with reference to the appended drawings.

### TESTS RELATING TO THE FIRST PREFERRED EMBODIMENT

A quantity of alumina fiber material of the type manufactured by Denki Kagaku Kogyo K.K. (Electrochemical Industries Company), with trade name "Denka-arusen", having a nominal composition of 80% by weight of Al<sub>2</sub>O<sub>3</sub> and 20% by weight of SiO<sub>2</sub>, with a quantity of non fibrous material intermingled therewith, was subjected to per se known particle elimination processing such as filtration or the like, so that the total amount of non fibrous particles included therein was brought to be about 0.8% by weight, and so that the included weight of non fibrous particles with a diameter greater than or equal to 150 microns included therein was brought to be about 0.05%. Thus, the parameters of this alumina fiber material were brought to be as shown in Table 1, which is given at the end of this specification and before the claims thereof.

Further, a quantity of mineral fiber material of the type manufactured by the Jim Walter Resources Company, with trade name "PMF" (Processed Mineral Fiber), having a nominal composition of 45% by weight of SiO<sub>2</sub>, 38% by weight of CaO, 9% by weight of Al<sub>2</sub>O<sub>3</sub>, 6% by weight of MgO, and remainder 2%, with a quantity of non fibrous material intermingled therewith, was similarly subjected to per se known particle elimination processing such as filtration or the like, so that the total amount of non fibrous particles included therein was brought to be about 2.5% by weight, and so that the included weight of non fibrous particles with a diameter greater than or equal to 150 microns included therein was brought to be about 0.1%; thus, the parameters of this mineral fiber material were brought to be as shown in Table 2, which is given at the end of this specification and before the claims thereof.

Next, using samples of these quantities of alumina fibers and of mineral fibers, there were formed eight preforms which will be designated as A0, A5, A10, A20, A40, A60, A80, and A100, in the following way. For each preform, first, a quantity of the alumina fibers with composition as per Table 1 and a quantity of the mineral fibers with composition as per Table 2 were dispersed together in colloidal silica, which acted as a binder: the relative proportions of the alumina fibers and of the mineral fibers were different in each case (and in one case no alumina fibers were utilized, while in another case no mineral fibers were utilized). In each case, the mixture was then well stirred up so that the alumina fibers and the mineral fibers were evenly dispersed therein and were well mixed together, and then the preform was formed by vacuum forming from the

5 mixture, said preform having dimensions of 80 by 80 by 20 millimeters, as shown in perspective view in FIG. 1, wherein it is designated by the reference numeral 1. As suggested in FIG. 1, the orientation of the alumina fibers 2 and of the mineral fibers 2a in these preforms 1 was not isotropic in three dimensions; in fact, the alumina fibers 2 and the mineral fibers 2a were largely oriented parallel to the longer sides of the cuboidal preforms 1, i.e. in the x-y plane as shown in FIG. 1, and were substantially randomly oriented in this plane; but the fibers 2 and 2a did not extend very substantially in the z direction as seen in FIG. 1, and were, so to speak, somewhat stacked on one another with regard to this direction. Finally, each preform was fired in a furnace at about 600° C., so that the silica bonded together the individual alumina fibers 2 and mineral fibers 2a, acting as a binder.

Next, a casting process was performed on each of the preforms, as schematically shown in section in FIG. 2. In turn, each of the preforms 1 was placed into the mold cavity 4 of a casting mold 3, and then a quantity of molten metal for serving as the matrix metal for the resultant composite material, in the case of this first preferred embodiment being molten aluminum alloy of type JIS (Japan Industrial Standard) AC8A and being heated to about 730° C., was poured into the mold cavity 4 over and around the preform 1. Then a piston 6, which closely cooperated with the defining surface of the mold cavity 4, was forced into said mold cavity 4 and was forced inwards, so as to pressurize the molten matrix metal to a pressure of about 1500 kg/cm<sup>2</sup> and thus to force it into the interstices between the fibers 2 and 2a of the preform 1. This pressure was maintained until the mass 5 of matrix metal was completely solidified, and then the resultant cast form 7, schematically shown in FIG. 3, was removed from the mold cavity 4. This cast form 7 was cylindrical, with diameter about 110 millimeters and height about 50 millimeters. Finally, heat treatment of type T7 was applied to the cast form 7, and from the part 1' of it (shown by phantom lines in FIG. 3) in which the fiber preform 1 was embedded was cut a test piece of composite material incorporating a mixture of alumina fibers and mineral fibers as the reinforcing fiber material and aluminum alloy as the matrix metal, of dimensions correspondingly again about 80 by 80 by 20 millimeters; thus, in all, eight such test pieces of composite material were manufactured, each corresponding to one of the preforms A0 through A100, and each of which will be hereinafter referred to by the reference symbol A0 through A100 of its parent preform since no confusion will arise therefrom. The parameters of these eight pieces of composite material are shown in Table 3, which is given at the end of this specification and before the claims thereof: in particular, for each composite material piece, the total volume proportion of the reinforcing fiber material is shown, along with the volume proportion of the alumina fibers and the volume proportion of the mineral fibers, the ratio between which is seen to be varied between zero and infinity. It will be seen from this table that the total reinforcing fiber volume proportion was substantially equal to about 20%, for each of the eight composite material sample pieces. As will be understood from the following, this set of test pieces included one or more preferred embodiments of the present invention and one or more comparison samples which were not embodiments of the present invention. From each of these test pieces was machined a wear test block sample, each of

which will also be hereinafter referred to by the reference symbol A0 through A100 of its parent preform.

In turn, each of these eight wear test sample pieces A0 through A100 was mounted in a LFW friction wear test machine, and its test surface was brought into contact with the outer cylindrical surface of a mating element, which was a cylinder of quench tempered bearing steel of type JIS (Japanese Industrial Standard) SUJ2, with hardness Hv equal to about 810. While supplying lubricating oil of type Castle Motor Oil (a trademark) and grade 5W-30 at the ambient temperature of about 20° C. to the contacting surfaces of the test pieces, in each case a friction wear test was carried out by rotating the cylindrical mating element for one hour, using a contact pressure of about 20 kg/mm<sup>2</sup> and a sliding speed of about 0.3 meters per second. It should be noted that in these wear tests the surface of the test piece which was contacted to the mating element was a plane perpendicular to the x—y plane as shown in FIG. 1.

The results of these friction wear tests are shown in FIG. 4. In this figure, which is a two sided graph, for each of the wear test samples A0 through A100, the upper half shows along the vertical axis the amount of wear on the actual test sample of composite material in microns, and the lower half shows along the vertical axis the amount of wear on the mating member (i.e., the bearing steel cylinder) in milligrams. And the volume proportion in percent of the total reinforcing fiber volume incorporated in said sample piece which consists of alumina fibers, i.e. the so called relative volume proportion of alumina fibers, is shown along the horizontal axis.

Now, from this FIG. 4, it will be understood that the wear amount of the test piece dropped along with increase in the relative volume proportion of alumina fibers incorporated in said test piece, and particularly dropped very quickly along with increase in said relative volume proportion when said relative volume proportion was in the range of 0% to about 20%, i.e. in the range of fairly low relative volume proportion of alumina fibers, but on the other hand had a relatively small variation with variation of said relative volume proportion when said relative volume proportion of alumina fibers was greater than about 20%. On the other hand, the wear amount of the mating member (the bearing steel cylinder) increased slightly with increase in said relative volume proportion of the alumina fibers, when said relative volume proportion was in the range of 0% to 20% or so, but, when said relative volume proportion was greater than about 20%, became substantially independent of said relative volume proportion, and was still fairly low, in all cases.

Now, it is sometimes maintained that the construction and composition of a composite material are subject to design criteria according to structural considerations. In such a case, the so called compounding rule would be assumed to hold. If this rule were to be applied to the present case, taking X% to represent the relative volume proportion of the alumina fibers incorporated in each of said test samples, as defined above, since when X% was equal to 0% the wear amount of the test sample piece was equal to about 98 microns, whereas when X% was equal to 100% the wear amount of the test sample piece was equal to about 5 microns, then by the compounding rule the wear amount Y of the block test piece for arbitrary values of X% would be determined by the equation:

$$Y = (98 - 15) \times / 100 + 5$$

This is just a linear fitting. Now, the double dotted line in FIG. 4 shows this linear approximation, and it is immediately visible that there is a great deviation dY between this linear approximation derived according to the compounding rule and the actual measured values for wear on the test samples. In short, the compounding rule is inapplicable, and this particular type of composite material at least is not subject to design criteria according to structural considerations.

In more detail, in FIG. 5, the value of this deviation dY between the linear approximations derived according to the compounding rule and the actual measured wear values is shown plotted on the vertical axis, while the relative volume proportion of the alumina fibers incorporated in the test samples is shown along the horizontal axis. From this figure, it is confirmed that when the relative volume proportion of the alumina fibers is in the range of 5% to 80%, and particularly when said relative volume proportion of the alumina fibers is in the range of 10% to 65%, the actual wear amount of the test sample piece is very much reduced from the wear amount value predicted by the compounding rule. This effect is thought to be due to the hybridization of the alumina fibers and the mineral fibers in this type of composite material. Accordingly, from these test results, it is considered that, from the point of view on a part or finished member made of the composite material according to the present invention, it is desirable that the relative volume proportion of the alumina fibers in the hybrid fiber mixture material incorporated as fibrous reinforcing material for the composite material according to this invention should be in the range of 5% to 80%, and preferably should be in the range of 10% to 65%.

#### TESTS RELATING TO THE SECOND PREFERRED EMBODIMENT

A quantity of alumina fiber material of the type used in the first preferred embodiment, manufactured by Denki Kagaku Kogyo K.K (Electrochemical Industries Company), with trade name "Denka-arusen", having a nominal composition of 80% by weight of Al<sub>2</sub>O<sub>3</sub> and 20% by weight of SiO<sub>2</sub>, with a quantity of non fibrous material intermingled therewith, was as before subjected to per se known particle elimination processing such as filtration or the like, so that the total amount of non fibrous particles included therein was brought to be about 0.8% by weight, and so that the included weight of non fibrous particles with a diameter greater than or equal to 150 microns included therein was brought to be about 0.05%. Thus, again the parameters of this alumina fiber material were brought to be as shown in Table 1. Further, a quantity of mineral fiber material of the type manufactured by Nitto Boseki KK, with trade name "Microfiber", having a nominal composition of 40% by weight of SiO<sub>2</sub>, 39% by weight of CaO, 15% by weight of Al<sub>2</sub>O<sub>3</sub>, and 6% by weight of MgO, with a quantity of non fibrous material intermingled therewith, was subjected to per se known particle elimination processing such as filtration or the like, so that the total amount of non fibrous particles was brought to be about 1.0% by weight, and so that the included weight of non fibrous particles with a diameter greater than or equal to 150 microns was about 0.1%; thus, the parameters of this mineral fiber material were as given in Table 4, which is

given at the end of this specification and before the claims thereof.

Next, using samples of these quantities of alumina fibers and of mineral fibers, there were formed six preforms which will be designated as B0, B20, B40, B60, B80, and B100, in a similar way to that practiced in the case of the first preferred embodiment described above. For each preform, first, a quantity of the alumina fibers with composition as per Table 1 and a quantity of the mineral fibers with composition as per Table 4 were dispersed together in colloidal silica, which acted as a binder, with the relative proportions of the alumina fibers and of the mineral fibers being different in each case. In each case, the mixture was then well stirred up so that the alumina fibers and the mineral fibers were evenly dispersed therein and were well mixed together, and then the preform as shown in FIG. 1 was formed by vacuum forming from the mixture, said preform again having dimensions of 80 by 80 by 20 millimeters. Again, in these preforms 1, the alumina fibers 2 and the mineral fibers 2a were largely oriented parallel to the longer sides of the cuboidal preforms 1, i.e. in the x—y plane as shown in FIG. 1, and were substantially randomly oriented in this plane. Finally, each preform was fired in a furnace at about 600° C., so that the silica bonded together the individual alumina fibers 2 and mineral fibers 2a, acting as a binder.

Next, as in the case of the first preferred embodiment, a casting process was performed on each of the preforms, as schematically shown in section in FIG. 2. In turn, each of the preforms 1 was placed into the mold cavity 4 of the casting mold 3, and then a quantity of molten metal for serving as the matrix metal for the resultant composite material, in the case of this second preferred embodiment again being molten aluminum alloy of type JIS (Japan Industrial Standard) AC8A and again being heated to about 730° C., was poured into the mold cavity 4 over and around the preform 1. Then a piston 6, which closely cooperated with the defining surface of the mold cavity 4, was forced into said mold cavity 4 and was forced inwards, so as to pressurize the molten matrix metal to a pressure again of about 1500 kg/cm<sup>2</sup> and thus to force it into the interstices between the fibers 2 and 2a of the preform 1. This pressure was maintained until the mass 5 of matrix metal was completely solidified, and then the resultant cast form 7, schematically shown in FIG. 3, was removed from the mold cavity 4. This cast form 7 was cylindrical, again with diameter about 110 millimeters and height about 50 millimeters. Finally, again, heat treatment of type T7 was applied to this cast form 7, and from the part of it (shown by phantom lines in FIG. 3) in which the fiber preform 1 was embedded was cut a test piece of composite material incorporating alumina fibers and mineral fibers as the reinforcing fiber material and aluminum alloy as the matrix metal, of dimensions correspondingly again about 80 by 80 by 20 millimeters; thus, in all, six such test pieces of composite material were manufactured, each corresponding to one of the preforms B0 through B100, and each of which will be hereinafter referred to by the reference symbol B0 through B100 of its parent preform since no confusion will arise therefrom. The parameters of these six pieces of composite material are shown in Table 5, which is given at the end of this specification and before the claims thereof: in particular, for each composite material piece, the total volume proportion of the reinforcing fiber material is shown, along with the volume proportion of the alu-

mina fibers and the volume proportion of the mineral fibers, the ratio between which is seen to be varied between zero and infinity. It will be seen from this table that the total reinforcing fiber volume proportion was substantially equal to about 3.5%, for each of the six composite material sample pieces. As will be understood from the following, this set of test pieces included one or more preferred embodiments of the present invention and one or more comparison samples which were not embodiments of the present invention. From each of these test pieces was machined a wear test block sample, each of which will also be hereinafter referred to by the reference symbol B0 through B100 of its parent preform.

In turn, each of these six wear test samples B0 through B100 was mounted in a LFW friction wear test machine, and was subjected to a wear test under the same test conditions as in the case of the first preferred embodiment described above, again using as mating member a steel cylinder. The results of these friction wear tests are shown in FIG. 6. In this figure, which is a two sided graph similar to the FIG. 4 graph for the first preferred embodiment, for each of the wear test samples B0 through B100, the upper half shows along the vertical axis the amount of wear on the actual test sample of composite material in microns, and the lower half shows along the vertical axis the amount of wear on the mating member (i.e., the steel cylinder) in milligrams. And the volume proportion in percent of the total reinforcing fiber volume incorporated in said sample pieces which consists of alumina fibers, i.e. the so called relative volume proportion of alumina fibers, is shown along the horizontal axis.

Now, from this FIG. 6, it will be understood that, also in this second preferred embodiment case, the wear amount of the test piece dropped along with increase in the relative volume proportion of the alumina fibers incorporated in said test piece, and particularly dropped very quickly along with increase in said relative volume proportion when said relative volume proportion was in the range of 0% to about 60%, i.e. in the range of fairly low relative volume proportion of alumina fibers, but on the other hand had a relatively small variation when said relative volume proportion of alumina fibers was greater than about 80%. On the other hand, the wear amount of the mating member (the steel cylinder) was substantially linearly dependent on the relative volume proportion of alumina fibers, and was fairly low in all cases.

Again, with reference to the so called compounding rule, if this rule were to be applied to the present case, the same type of linear fitting as before, as shown in FIG. 6 by the double dotted line, would be obtained. Again, it is immediately visible that there is a great deviation dY between this linear approximation derived according to the compounding rule and the actual measured values for wear on the test samples. In FIG. 7, the value of this deviation dY between the linear approximation derived according to the compounding rule and the actual measured wear values for this second preferred embodiment is shown plotted on the vertical axis, while the relative volume proportion of the alumina fibers incorporated in the test samples is shown along the horizontal axis. From this figure is confirmed that, when the relative volume proportion of the alumina fibers is in the range of 10% to 80%, the actual wear amount of the test sample piece is very much reduced from the wear amount value predicted by the com-

pounding rule. Again, this effect is thought to be due to the hybridization of the alumina fibers and the mineral fibers in this type of composite material.

### THE THIRD PREFERRED EMBODIMENT USE OF MAGNESIUM ALLOY MATRIX METAL

A quantity of alumina fiber material of the type manufactured by ICI K.K. with trade name "Saffil", having a nominal composition of 95% by weight of  $Al_2O_3$  and 5% by weight of  $SiO_2$ , with a quantity of non fibrous material intermingled therewith, was subjected to per se known particle elimination processing such as filtration or the like, so that the total amount of non fibrous particles included therein was brought to be about 1% by weight, and so that the included weight of non fibrous particles with a diameter greater than or equal to 150 microns included therein was brought to be about 0.1%. The alpha alumina content of this alumina fiber material was about 55% by weight. Thus, the parameters of this alumina fiber material were brought to be as shown in Table 6, which is given at the end of this specification and before the claims thereof.

Further, a quantity of mineral fiber material of the type used in the second preferred embodiment described above, manufactured by Nitto Boseki KK, with trade name "Microfiber", having a nominal composition of 40% by weight of  $SiO_2$ , 39% by weight of  $CaO$ , 15% by weight of  $Al_2O_3$ , and 6% by weight of  $MgO$ , with a quantity of non fibrous material intermingled therewith, was subjected to per se known particle elimination processing such as filtration or the like, as in the case of said second preferred embodiment, so as to have parameters as given in Table 4 mentioned above.

Next, using samples of these quantities of alumina fibers and of mineral fibers, there were formed seven preforms which will be designated as C0, C10, C20, C40, C60, C80, and C100, in similar ways to those practiced in the case of the first preferred embodiment described above. As before, for each preform, a quantity of the alumina fibers with composition as per Table 6 and a quantity of the mineral fibers with composition as per Table 4 were well and evenly mixed together in colloidal silica in various different volume proportions, and then the preform as shown in FIG. 1 was formed by vacuum forming from the mixture, said preform again having dimensions of 80 by 80 by 20 millimeters. Again, in these preforms 1, the alumina fibers 2 and the mineral fibers 2a were largely oriented parallel to the longer sides of the cuboidal preforms 1, i.e. in the x-y plane as shown in FIG. 1, and were substantially randomly oriented in this plane. Finally, again, each preform was fired in a furnace at about 600° C., so that the silica bonded together the individual alumina fibers 2 and mineral fibers 2a, acting as a binder.

Next, as in the case of the first and second preferred embodiments, a casting process was performed on each of the preforms, as schematically shown in FIG. 2, using as the matrix metal for the resultant composite material, in the case of this third preferred embodiment, molten magnesium alloy of type JIS (Japan Industrial Standard) AZ91, which in this case was heated to about 690° C., and pressurizing this molten matrix metal by the piston 6 to a pressure again of about 1500 kg/cm<sup>2</sup>, so as to force it into the interstices between the fibers 2 and 2a of the preform 1. This pressure was maintained until the mass 5 of matrix metal was completely solidified, and then the resultant cast form 7, again as schematically shown in FIG. 3, was removed from the mold

cavity 4. This cast form 7 again was cylindrical, with diameter about 110 millimeters and height about 50 millimeters. Finally, again, from the part of this cast form 7 (shown by phantom lines in FIG. 3) in which the fiber preform 1 was embedded was cut a test piece of composite material incorporating alumina fibers and mineral fibers as the reinforcing fiber material and magnesium alloy as the matrix metal, of dimensions correspondingly again about 80 by 80 by 20 millimeters; thus, in all, this time, seven such test pieces of composite material were manufactured, each corresponding to one of the preforms C0 through C100, and each of which will be hereinafter referred to by the reference symbol C0 through C100 of its parent preform since no confusion will arise therefrom. The parameters of these seven pieces of composite material are shown in Table 7, which is given at the end of this specification and before the claims thereof: in particular, for each composite material piece, the total volume proportion of the reinforcing fiber material is shown, along with the volume proportion of the alumina fibers and the volume proportion of the mineral fibers, the ratio between which is seen to be varied between zero and infinity. It will be seen from this table that the total reinforcing fiber volume proportion was substantially equal to about 8%, for each of the seven composite material sample pieces. As will be understood from the following, this set of test pieces included one or more preferred embodiments of the present invention and one or more comparison samples which were not embodiments of the present invention. From each of these test pieces was machined a wear test block sample, each of which will also be hereinafter referred to by the reference symbol C0 through C100 of its parent preform.

In turn, each of these seven wear test samples C0 through C100 was mounted in a LFW friction wear test machine, and was subjected to a wear test under the same test conditions as in the case of the first preferred embodiment described above, using as in the case of that embodiment a mating element which was a cylinder of bearing steel of type JIS (Japanese Industrial Standard) SUJ2, with hardness Hv equal to about 810. The results of these friction wear tests are shown in FIG. 8. In this figure, which is a two sided graph similar to the graphs of FIGS. 4 and 6, for each of the wear test samples C0 through C100, the upper half shows along the vertical axis the amount of wear on the actual test sample of composite material in microns, and the lower half shows along the vertical axis the amount of wear on the mating member (i.e., the bearing steel cylinder) in milligrams. And the volume proportion in percent of the total reinforcing fiber volume incorporated in said sample pieces which consists of alumina fibers, i.e. the so called relative volume proportion of alumina fibers, is shown along the horizontal axis.

Now, from this FIG. 8, it will be understood that, also in this third preferred embodiment, the wear amount of the test piece dropped along with increase in the relative volume proportion of the alumina fibers incorporated in said test piece, and particularly dropped very quickly along with increase in said relative volume proportion when said relative volume proportion was in the range of 0% to about 40%, i.e. in the range of fairly low relative volume proportion of alumina fibers, but on the other hand had a relatively small variation when said relative volume proportion of alumina fibers was greater than about 60%. On the other hand, the wear

amount of the mating member (the bearing steel cylinder) was substantially independent of the relative volume proportion of alumina fibers, and was fairly low in all cases.

Again, with reference to the so called compounding rule, if this rule were to be applied to the present case, the same type of linear fitting as shown in FIG. 8 by the double dotted line would be obtained. Again, it is immediately visible that there is a great deviation  $dY$  between this linear approximation derived according to the compounding rule and the actual measured values for wear on the test samples. In FIG. 9 (similarly to FIGS. 5 and 7), the value of this deviation  $dY$  between the linear approximation derived according to the compounding rule and the actual measured wear values for this third preferred embodiment is shown plotted on the vertical axis, while the relative volume proportion of the alumina fibers incorporated in the test samples is shown along the horizontal axis. From this figure is confirmed that, when the relative volume proportion of the alumina fibers is in the range of from 5% to 80%, and even more when said relative volume proportion is in the range of from 10% to 70%, the actual wear amount of the test sample piece is very much reduced from the wear amount value predicted by the compounding rule. Again, this effect is thought to be due to the hybridization of the alumina fibers and the mineral fibers in this type of composite material.

#### TESTS RELATING TO THE FOURTH PREFERRED EMBODIMENT

A quantity of alumina fiber material which was another version of the type manufactured by ICI K.K., with trade name "Saffil", having a nominal composition of 95% by weight of  $Al_2O_3$  and 5% by weight of  $SiO_2$ , with a quantity of non fibrous material intermingled therewith, was subjected to per se known particle elimination processing such as filtration or the like, so that the total amount of non fibrous particles included therein was brought to be about 1% by weight, and so that the included weight of non fibrous particles with a diameter greater than or equal to 150 microns included therein was brought to be about 0.1%. The crystalline structure of these alumina fibers was the delta crystalline structure. Thus, the parameters of this alumina fiber material were brought to be as shown in Table 8, which is given at the end of this specification and before the claims thereof.

Further, a quantity of mineral fiber material of the type used in the second and third preferred embodiments described above, manufactured by Nitto Boseki K.K., with trade name "Microfiber", having a nominal composition of 40% by weight of  $SiO_2$ , 39% by weight of  $CaO$ , 15% by weight of  $Al_2O_3$ , and 6% by weight of  $MgO$ , with a quantity of non fibrous material intermingled therewith, was subjected to per se known particle elimination processing such as filtration or the like, as in the case of said second preferred embodiment, so as again to have parameters as given in Table 4 mentioned above.

Next, using samples of these quantities of alumina fibers and of mineral fibers, these were formed seven preforms which will be designated as D0, D10, D20, D40, D60, D80, and D100, in similar ways to those practiced in the case of the first preferred embodiment described above. As before, for each preform, a quantity of the alumina fibers with composition as per Table 8 and a quantity of the mineral fibers with composition

as per Table 4 were well and evenly mixed together in colloidal silica in various different volume proportions, and then the preform as shown in FIG. 1 was formed by vacuum forming from the mixture, said preform again having dimensions of 80 by 80 by 20 millimeters. Again, in these preforms 1, the alumina fibers 2 and the mineral fibers 2a, were largely oriented parallel to the longer sides of the cuboidal preforms 1, i.e. in the x-y plane as shown in FIG. 1, and were substantially randomly oriented in this plane. Finally, again, each preform was fired in a furnace at about 600° C., so that the silica bonded together the individual alumina fibers 2 and mineral fibers 2a, acting as a binder.

Next, as in the case of the first and second preferred embodiments, a casting process was performed on each of the preforms, as schematically shown in FIG. 2, using as the matrix metal for the resultant composite material, in the case of this fourth preferred embodiment, molten magnesium alloy of type JIS (Japan Industrial Standard) AZ91, which in this case was heated to about 690° C., and pressurizing this molten matrix metal by the piston 6 to a pressure again of about 1500 kg/cm<sup>2</sup>, so as to force it into the interstices between the fibers 2 and 2a of the preform 1. This pressure was maintained until the mass 5 of matrix metal was completely solidified, and then the resultant cast form 7, schematically shown in FIG. 3, was removed from the mold cavity 4. This cast form 7 again was cylindrical, with diameter about 110 millimeters and height about 50 millimeters. Finally, again, from the part of this cast form 7 (shown by phantom lines in FIG. 3) in which the fiber preform 1 was embedded was cut a test piece of composite material incorporating alumina fibers and magnesium alloy as the matrix metal, of dimensions correspondingly again about 80 by 80 by 20 millimeters; thus, in all, this time, seven such test pieces of composite material were manufactured, each corresponding to one of the preforms D0 through D100, and each of which will be hereinafter referred to by the reference symbol D0 through D100 of its parent preform since no confusion will arise therefrom. The parameters of these seven pieces of composite material are shown in Table 9, which is given at the end of this specification and before the claims thereof: in particular, for each composite material piece, the total volume proportion of the reinforcing fiber material is shown, along with the volume proportion of the alumina fibers and the volume proportion of the mineral fibers, the ratio between which is seen to be varied between zero and infinity. It will be seen from this table that the total reinforcing fiber volume proportion was substantially equal to about 8%, for each of the seven composite material sample pieces. As will be understood from the following, this set of test pieces included one or more preferred embodiments of the present invention and one or more comparison samples which were not embodiments of the present invention. From each of these test pieces was machined a wear test block sample, each of which will also be hereinafter referred to by the reference symbol D0 through D100 of its parent preform.

In turn, each of these seven wear test samples D0 through D100 was mounted in a LFW friction wear test machine, and was subjected to a wear test under the same test conditions as in the case of the first preferred embodiment described above, using as in the case of that embodiment a mating element which was a cylinder of quench tempered bearing steel of type JIS (Japa-

nese Industrial Standard) SUJ2, with hardness Hv equal to about 810. The results of these friction wear tests are shown in FIG. 10. In this figure, which is a two sided graph similar to FIGS. 4, 6, and 8, for each of the wear test samples D0 through D100, the upper half shows along the vertical axis the amount of wear on the actual test sample of composite material in microns, and the lower half shows along the vertical axis the amount of wear on the mating member (i.e., the bearing steel cylinder) in milligrams. And the volume proportion in percent of the total reinforcing fiber volume incorporated in said sample pieces which consists of alumina fibers, i.e. the so called relative volume proportion of alumina fibers, is shown along the horizontal axis.

Now, from this FIG. 8, it will be understood that, also in this fourth preferred embodiment, the wear amount of the test piece dropped along with increase in the relative volume proportion of the alumina fibers incorporated in said test piece, and particularly dropped very quickly along with increase in said relative volume proportion when said relative volume proportion was in the range of 0% to about 40%, i.e. in the range of fairly low relative volume proportion of alumina fibers, but on the other hand had a relatively small variation when said relative volume proportion of alumina fibers was greater than about 60%. On the other hand, the wear amount of the mating member (the bearing steel cylinder) was, as in the case of the third preferred embodiment described above, substantially independent of the relative volume proportion of alumina fibers, and was fairly low in all cases.

Again, with reference to the so called compounding rule, if this rule were to be applied to the present case, the same type of linear fitting as shown in FIG. 10 by the double dotted line would be obtained. Again, it is immediately visible that there is a great deviation  $dY$  between this linear approximation derived according to the compounding rule and the actual measured values for wear on the test samples. In FIG. 11, which is a graph similar to the graphs of FIGS. 5, 7, and 9, the value of this deviation  $dY$  between the linear approximation derived according to the compounding rule and the actual measured wear values for this fourth preferred embodiment is shown plotted on the vertical axis, while the relative volume proportion of the alumina fibers incorporated in the test samples is shown along the horizontal axis. From this figure is confirmed that, when the relative volume proportion of the alumina fibers is in the range of from 5% to 80%, and even more when said relative volume proportion is in the range of from 10% to 70%, the actual wear amount of the test sample piece is very much reduced from the wear amount value predicted by the compounding rule. Again, this effect is thought to be due to the hybridization of the alumina fibers and the mineral fibers in this type of composite material.

#### TESTS RELATING TO THE FIFTH PREFERRED EMBODIMENT

#### BENDING STRENGTH TESTS

A quantity of alumina fiber material of the type utilized in the fourth preferred embodiment described above, manufactured by ICI K.K with trade name "Safil", having a nominal composition of 95% by weight of  $Al_2O_3$  and 5% by weight of  $SiO_2$ , with a quantity of non fibrous material intermingled therewith, was subjected to per se known particle elimination processing such as filtration or the like, so that the total amount of non

fibrous particles included therein was brought to be about 1% by weight, and so that the included weight of non fibrous particles with a diameter greater than or equal to 150 microns included therein was brought to be about 0.1%. The crystalline structure of these alumina fibers was the delta crystalline structure. Thus, the parameters of this alumina fiber material were brought to be as shown in Table 8 above. Further, a quantity of mineral fiber material also of the type used in the second through the fourth preferred embodiments described above, manufactured by Nitto Boseki KK, with trade name "Microfiber", having a nominal composition of 40% by weight of  $SiO_2$ , 39% by weight of  $CaO$ , 15% by weight of  $Al_2O_3$ , and 6% by weight of  $MgO$ , with a quantity of non fibrous material intermingled therewith, was subjected to per se known particle elimination processing such as filtration or the like, as in the case of said second preferred embodiment, so as to have parameters as given in Table 4 mentioned above.

Next, using samples of these quantities of alumina fibers and of mineral fibers, there were formed seven preforms which will be designated as E0, E10, E20, E40, E60, E80, and E100, in similar ways to those practiced in the case of the first through the third preferred embodiments described above. As before, for each preform, quantity of the alumina fibers with composition as per Table 8 and a quantity of the mineral fibers with composition as per Table 4 were well and evenly mixed together in colloidal silica in various different volume proportions, and then the preform as shown in FIG. 1 was formed by vacuum forming from the mixture, said preform again having dimensions of 80 by 80 by 20 millimeters. Again, in these preforms 1, the alumina fibers 2 and the mineral fibers 2a were largely oriented parallel to the longer sides of the cuboidal preforms 1, i.e. in the x-y plane as shown in FIG. 1, and were substantially randomly oriented in this plane. Finally, again, each preform was fired in a furnace at about 600°C., so that the silica bonded together the individual alumina fibers 2 and mineral fibers 2a, acting as a binder.

Next, as in the case of the first through the third preferred embodiments, a casting process was performed on each of the preforms, as schematically shown in FIG. 2, using as the matrix metal for the resultant composite material, in the case of this fifth preferred embodiment, molten aluminum alloy of type JIS (Japan Industrial Standard) AC8A, which in this case was heated to about 730°C., and pressurizing this molten matrix metal by the piston 6 to a pressure again of about 1500 kg/cm<sup>2</sup>, so as to force it into the interstices between the fibers 2 and 2a of the preform 1. This pressure was maintained until the mass 5 of matrix metal was completely solidified, and then the resultant cast form 7, schematically shown in FIG. 3, was removed from the mold cavity 4. This cast form 7 again was cylindrical, with diameter about 110 millimeters and height about 50 millimeters. Finally, again, heat treatment of type T7 was applied to this cast form 7, and from the part of it (shown by phantom lines in FIG. 3) in which the fiber preform 1 was embedded was cut a test piece of composite material incorporating alumina fibers and mineral fibers as the reinforcing fiber material and aluminum alloy as the matrix metal, of dimensions correspondingly again about 80 by 80 by 20 millimeters; thus, in all, this time, seven such test pieces of composite material were manufactured, each corresponding to one of the preforms E0 through E100, and each of which will be

hereinafter referred to by the reference symbol E0 through E100 of its parent preform since no confusion will arise therefrom. The parameters of these seven pieces of composite material are shown in Table 10, which is given at the end of this specification and before the claims thereof; in particular, for each composite material piece, the total volume proportion of the reinforcing fiber material is shown, along with the volume proportion of the alumina fibers and the volume proportion of the mineral fibers, the ratio between which is seen to be varied between zero and infinity. It will be seen from this table that the total reinforcing fiber volume proportion was substantially equal to about 8%, for each of the seven composite material sample pieces. As will be understood from the following, this set of test pieces included one or more preferred embodiments of the present invention and one or more comparison samples which were not embodiments of the present invention. From each of these test pieces was machined a bending strength test block sample, each of which will also be hereinafter referred to by the reference symbol E0 through E100 of its parent preform. Each of these bending strength test samples had dimensions about 50 mm by 10 mm by 2 mm, and its 50 mm by 10 mm surface was cut parallel to the x-y plane as seen in FIG. 1 of the composite material mass.

Next, each of these bending strength test samples E0 through E100 was subjected to a three point bending test at a temperature of about 350° C., with the gap between the support ports being set to about 39 mm. Also, for purposes of comparison, a similar bending test was carried out upon a similarly cut piece of pure matrix metal, i.e. of aluminum alloy of type JIS (Japan Industrial Standard) AC8A to which heat treatment of type T7 had been applied. The bending strength in each case was measured as the surface stress at breaking point of the test piece M/Z (M is the bending moment at breaking point, and Z is the cross sectional coefficient of the bending strength test sample piece). The results of these bending strength tests are shown in FIG. 12, which is a graph showing bending strength for each of the seven bending test samples E0 through E100 and for the comparison test sample piece, with the volume proportion in percent of the total reinforcing fiber volume incorporated in said bending strength test sample pieces which consists of alumina fibers, i.e. the so called relative volume proportion of alumina fibers, shown along the horizontal axis, and with the corresponding bending strength in kg/mm<sup>2</sup> shown along the vertical axis.

From this graph in FIG. 12, it will be apparent that, even in this case when the total volume proportion of the reinforcing fibers was relatively low and equal to about 8%, nevertheless the bending strength of the test sample pieces was relatively high, much higher than that of the comparison piece made of matrix metal on its own. It will also be understood that the bending strength of the test sample pieces was roughly linearly related to the relative volume proportion of alumina fibers included therein.

#### TESTS RELATING TO THE SIXTH PREFERRED EMBODIMENT

##### THE USE OF OTHER MATRIX METALS

In the same way and under the same conditions as in the case of the first preferred embodiment described above, a quantity of alumina fiber material of the type manufactured by Denki Kagaku Kogyo K.K (Electro-chemical Industries Company), with trade name "Den-

ka-arusen", having a nominal composition of 80% by weight of Al<sub>2</sub>O<sub>3</sub> and 20% by weight of SiO<sub>2</sub>, with a quantity of non fibrous material intermingled therewith, was subjected to particle elimination processing, so that the total amount of non fibrous particles was brought to be about 0.8% by weight, and so that the included weight percent of non fibrous particles with a diameter greater than or equal to 150 microns was reduced to be equal to about 0.05%; thus the parameters of this alumina fiber material were brought to be as shown in Table 1. Further, as in the first preferred embodiment, a quantity of mineral fiber material of the type manufactured by the Jim Walter Resources Company, with trade name "PMF" (Processed Mineral Fiber), having a nominal composition of 45% by weight of SiO<sub>2</sub>, 38% by weight of CaO, 9% by weight of Al<sub>2</sub>O<sub>3</sub>, 6% by weight of MgO, and remainder 2%, with a quantity of non fibrous material intermingled therewith, was subjected to per se known particle elimination processing such as filtration or the like, so that the total amount of non fibrous particles was brought to be about 2.5% by weight, and so that the included weight percentage of non fibrous particles with a diameter greater than or equal to 150 microns was about 0.1%; thus, the parameters of this mineral fiber material were brought to be as given in Table 2. Next, quantities of these two fiber materials were mixed together in colloidal silica as in the case of the first preferred embodiment, and from this mixture three preforms were formed by the vacuum forming method, said preforms again having dimensions of 80 by 80 by 20 millimeters as before, and as before the preforms were fired in a furnace at about 600° C. The fiber volume proportion for each of these three preforms was about 15%, and the relative volume proportion of the alumina fibers was about 20% in each case. And then high pressure casting processes were performed on the preforms, in substantially the same way as in the case described above of the first preferred embodiment, but this time using a pressure of only about 500 kg/cm<sup>2</sup> as the casting pressure in each case, and respectively using as the matrix metal zinc alloy of type JIS (Japanese Industrial Standard) ZDC1, pure lead (of purity 99.8%), and tin alloy of type JIS (Japanese Industrial Standard) WJ2, which are molten by being respectively heated to casting temperatures of about 500° C., about 410° C., and about 330° C. From the parts of the resulting cast masses in which the fiber preforms were embedded were then machined wear test samples of composite material incorporating a mixture of alumina fibers and mineral fibers as the reinforcing fiber material and, respectively, zinc alloy, pure lead, and tin alloy as the matrix metal.

Then these wear samples were tested in substantially the same way and under the same operational conditions as in the case of the first preferred embodiment described above (except that the contact pressure was 5 kg/mm<sup>2</sup> and the period of test was about 30 minutes), using as the mating element a cylinder of bearing steel of type JIS (Japanese Industrial Standard) SUJ2, with hardness Hv equal to about 810. The results of these friction wear tests were that the amounts of wear on the test samples of these composite materials were respectively about 4%, about 1%, and about 2% of the wear amounts on comparison test sample pieces made of only the corresponding matrix metal without any reinforcing fibers. Accordingly, it is concluded that by using this mixed reinforcing fiber material made up from alumina

fiber material and mineral fiber material as the fibrous reinforcing material for the composite material, also in these cases of using zinc alloy, lead, or tin alloy as matrix metal, the characteristics of the composite material with regard to wear resistance are very much improved, as compared to the characteristics of pure matrix metal only.

Although the present invention has been shown and described with reference to these preferred embodiments thereof, in terms of a portion of the experimental research carried out by the present inventors, and in terms of the illustrative drawings, it should not be considered as limited thereby. Various possible modifications, omissions, and alterations could be conceived of by one skilled in the art to the form and the content of any particular embodiment, without departing from the scope of the present invention. Therefore, it is desired that the scope of the present invention, and the protection sought to be granted by Letters Patent, should be defined not by any of the perhaps purely fortuitous details of the shown preferred embodiments, or of the drawings, but solely by the scope of the appended claims, which follow.

TABLE I

|                                                                                         |                                                            |
|-----------------------------------------------------------------------------------------|------------------------------------------------------------|
| Chemical composition (wt %)                                                             | Al <sub>2</sub> O <sub>3</sub> :80%, SiO <sub>2</sub> :20% |
| Average fiber diameter (microns)                                                        | 2.9                                                        |
| Average fiber length (mm)                                                               | 0.1                                                        |
| Total amount of non fibrous particles (wt %)                                            | 0.8                                                        |
| Amount of non fibrous particles of diameter greater than or equal to 150 microns (wt %) | 0.05                                                       |

TABLE 2

|                                                                                         |                                                                                          |
|-----------------------------------------------------------------------------------------|------------------------------------------------------------------------------------------|
| Chemical composition (wt %)                                                             | SiO <sub>2</sub> :45%, CaO:38%, Al <sub>2</sub> O <sub>3</sub> :9%, MgO:6%, remainder 2% |
| Average fiber diameter (microns)                                                        | 5                                                                                        |
| Average fiber length (mm)                                                               | 0.15                                                                                     |
| Total amount of non fibrous particles (wt %)                                            | 2.5                                                                                      |
| Amount of non fibrous particles of diameter greater than or equal to 150 microns (wt %) | 0.1                                                                                      |

TABLE 3

| Composite material sample                         | A0   | A5   | A10  | A20  | A40  | A60  | A80  | A100 |
|---------------------------------------------------|------|------|------|------|------|------|------|------|
| Total volume proportion of reinforcing fibers (%) | 20.0 | 20.0 | 20.1 | 20.0 | 20.1 | 20.0 | 19.9 | 20.0 |
| Volume proportion of alumina fibers (%)           | 0    | 1.0  | 2.0  | 4.0  | 8.1  | 11.9 | 15.9 | 20.0 |
| Volume proportion of mineral fibers (%)           | 20   | 19   | 18.1 | 16.0 | 12.0 | 8.1  | 4.0  | 0    |

TABLE 3-continued

| Composite material sample | A0                                 | A5 | A10 | A20 | A40 | A60 | A80 | A100 |
|---------------------------|------------------------------------|----|-----|-----|-----|-----|-----|------|
| Matrix metal              | Aluminum alloy (JIS standard AC8A) |    |     |     |     |     |     |      |

TABLE 4

|                                                                                         |                                                                             |
|-----------------------------------------------------------------------------------------|-----------------------------------------------------------------------------|
| Chemical composition (wt %)                                                             | SiO <sub>2</sub> :40%, CaO:39%, Al <sub>2</sub> O <sub>3</sub> :15%, MgO:6% |
| Average fiber diameter (microns)                                                        | 4.9                                                                         |
| Average fiber length (mm)                                                               | 5                                                                           |
| Total amount of non fibrous particles (wt %)                                            | 1.0                                                                         |
| Amount of non fibrous particles of diameter greater than or equal to 150 microns (wt %) | 0.1                                                                         |

TABLE 5

| Composite material sample                         | B0                                 | B20 | B40 | B60 | B80 | B100 |
|---------------------------------------------------|------------------------------------|-----|-----|-----|-----|------|
| Total volume proportion of reinforcing fibers (%) | 3.5                                | 3.4 | 3.5 | 3.5 | 3.6 | 3.5  |
| Volume proportion of alumina fibers (%)           | 0                                  | 0.7 | 1.4 | 2.1 | 2.9 | 3.5  |
| Volume proportion of mineral fibers (%)           | 3.5                                | 2.7 | 2.1 | 1.4 | 0.7 | 0    |
| Matrix metal                                      | Aluminum alloy (JIS standard AC8A) |     |     |     |     |      |

TABLE 6

|                                                                                         |                                                           |
|-----------------------------------------------------------------------------------------|-----------------------------------------------------------|
| Chemical composition (wt %)                                                             | Al <sub>2</sub> O <sub>3</sub> :95%, SiO <sub>2</sub> :5% |
| Average fiber diameter (microns)                                                        | 2.9                                                       |
| Average fiber length (mm)                                                               | 2                                                         |
| Total amount of non fibrous particles (wt %)                                            | 1                                                         |
| Amount of non fibrous particles of diameter greater than or equal to 150 microns (wt %) | 0.1                                                       |
| Alpha alumina content (wt %)                                                            | 55                                                        |

TABLE 7

| Composite material sample                         | C0                                   | C10 | C20 | C40 | C60 | C80 | C100 |
|---------------------------------------------------|--------------------------------------|-----|-----|-----|-----|-----|------|
| Total volume proportion of reinforcing fibers (%) | 8.0                                  | 8.1 | 8.1 | 8.0 | 7.9 | 8.0 | 7.9  |
| Volume proportion of alumina fibers (%)           | 0                                    | 0.8 | 1.6 | 3.2 | 4.7 | 6.4 | 7.9  |
| Volume proportion of mineral fibers (%)           | 8.0                                  | 8.7 | 6.5 | 4.8 | 3.2 | 1.6 | 0    |
| Matrix metal                                      | Magnesium alloy (ASTM standard AZ91) |     |     |     |     |     |      |

TABLE 8

|                                       |                                                           |
|---------------------------------------|-----------------------------------------------------------|
| Chemical composition (wt %)           | Al <sub>2</sub> O <sub>3</sub> :95%, SiO <sub>2</sub> :5% |
| Average fiber diameter (microns)      | 2.9                                                       |
| Average fiber length (mm)             | 1.5                                                       |
| Total amount of non fibrous particles | 1                                                         |

TABLE 8-continued

|                                                                                  |       |     |
|----------------------------------------------------------------------------------|-------|-----|
| (wt %)                                                                           |       | 0.1 |
| Amount of non fibrous particles of diameter greater than or equal to 150 microns |       |     |
| (wt %)                                                                           |       |     |
| Crystalline structure                                                            | Delta |     |

TABLE 9

| Composite material sample                         | D0                                   | D10 | D20 | D40 | D60 | D80 | D100 |
|---------------------------------------------------|--------------------------------------|-----|-----|-----|-----|-----|------|
| Total volume proportion of reinforcing fibers (%) | 8.0                                  | 8.0 | 8.1 | 8.1 | 7.9 | 8.0 | 8.1  |
| Volume proportion of alumina fibers (%)           | 0                                    | 0.8 | 1.6 | 3.3 | 4.7 | 7.2 | 8.1  |
| Volume proportion of mineral fibers (%)           | 8.0                                  | 7.2 | 6.5 | 4.8 | 3.2 | 0.8 | 0    |
| Matrix metal                                      | Magnesium alloy (ASTM standard AZ91) |     |     |     |     |     |      |

TABLE 10

| Composite material sample                         | E0                                 | E10 | E20 | E40 | E60 | E80 | E100 |
|---------------------------------------------------|------------------------------------|-----|-----|-----|-----|-----|------|
| Total volume proportion of reinforcing fibers (%) | 8.0                                | 8.0 | 8.1 | 8.1 | 7.9 | 8.0 | 8.1  |
| Volume proportion of alumina fibers (%)           | 0                                  | 0.8 | 1.6 | 3.3 | 4.7 | 7.2 | 8.1  |
| Volume proportion of mineral fibers (%)           | 8.0                                | 7.2 | 6.5 | 4.8 | 3.2 | 0.8 | 0    |
| Matrix metal                                      | Aluminum alloy (JIS standard AC8A) |     |     |     |     |     |      |

What is claimed is:

1. A composite material, consisting essentially of:
  - (a) a reinforcing material which is a hybrid fiber mixture material consisting essentially of:
    - (a1) an effective amount of a reinforcing alumina fiber material with the principal components being at least about 80% by weight of  $\text{Al}_2\text{O}_3$  and the remainder substantially  $\text{SiO}_2$ ; and
    - (a2) an effective amount of a reinforcing mineral fiber material having as the principal components  $\text{SiO}_2$ ,  $\text{CaO}$ , and  $\text{Al}_2\text{O}_3$ , the content of included  $\text{MgO}$  therein being less than or equal to about 10% by weight, the content of included  $\text{Fe}_2\text{O}_3$  therein being less than or equal to about 5% by weight, and the content of other inorganic substances included therein being less than or equal to about 10% by weight, with the percentage of non-fibrous particles included therein being less than or equal to about 20% by weight, and with the percentage of non-fibrous particles with diameters greater than about 150 microns included therein being less than or equal to about 7% by weight; and
    - (b) a matrix metal selected from the group consisting of aluminum, magnesium, copper, zinc, lead, tin, and alloys having these metals as principal components; and wherein

the volume proportion of said hybrid fiber mixture material in said composite material is at least 1%.

2. The composite material according to claim 1, wherein the alpha alumina content by weight of said alumina fiber material is between about 5% and about 60%.

3. The composite material according to claim 1, wherein the ratio of the volume proportion of said alumina fiber material to the total volume proportion of said hybrid fiber mixture material is between about 5% and about 80%.

4. The composite material according to claim 2, wherein the ratio of the volume proportion of said alumina fiber material to the total volume proportion of said hybrid fiber mixture material is between about 5% and about 40%, and the total volume proportion of said hybrid fiber mixture material is between about 2% and about 40%.

5. The composite material according to claim 1, wherein the volume proportion of said mineral fiber material in said composite material is less than or equal to about 25%.

6. The composite material according to claim 1, wherein the total proportion of non fibrous particles included in said mineral fiber material is less than or equal to about 10% by weight, and the proportion of non fibrous particles with diameters greater than about 150 microns included in said mineral fiber material is less than or equal to about 2% by weight.

7. The composite material according to claim 1, wherein the alpha alumina content by weight of said alumina fiber material is between about 10% and about 50%.

8. The composite material according to claim 1, wherein, in said hybrid fiber mixture material, said alumina fiber material and said mineral fiber material are substantially evenly mixed together.

9. The composite material according to claim 1, wherein said matrix metal is an aluminum alloy.

10. The composite material according to claim 1, wherein said matrix metal is a magnesium alloy.

11. The composite material according to claim 1, wherein said matrix metal is a zinc alloy.

12. The composite material according to claim 1, wherein said matrix metal is lead.

13. The composite material according to claim 1, wherein said matrix metal is a tin alloy.

14. The composite material according to claim 1, wherein said alumina fibers are short fibers having an average fiber diameter of approximately 1.5 to 5.0 microns and a fiber length of 20 microns to 3 mm.

15. The composite material according to claim 1, wherein said alumina fibers are long fibers having an average fiber diameter of approximately 3 to 30 microns.

16. The composite material according to claim 1, wherein said mineral fibers are in the form of short fibers with a fiber diameter of about 1 to 10 microns and with a fiber length of about 10 microns to about 10 cm.

\* \* \* \* \*